# EUROPEAN PATENT APPLICATION

(11) **EP 0 787 817 A2**
(43) Date of publication of application: **06.08.1997**
(21) Application number: 96302671.1
(22) Date of filing: 17.04.1996
(51) Int. Cl.: C23C 8/02, C23C 8/34

(54) **Method of carburizing austenitic stainless steel and austenitic stainless steel products obtained thereby**

(30) Priority: 30.01.1996 JP 14365/96
(71) Applicant: DAIDO HOXAN INC., Sapporo-shi, Hokkaido 060 (JP)
(72) Inventor: Tahara, Masaaki, Takatsuki-shi, Osaka 569 (JP); Senbokuya, Haruo, Tondabayashi-shi, Osaka 584 (JP); Kitano, Kinzo, Kawachinagano-shi, Osaka 586 (JP); Hayashida, Tadashi, Nishinomiya-shi, Hyogo 662 (JP)
(74) Representative: Wakerley, Helen Rachael

(57) **Abstract**

A method of carburizing austenitic stainless steel comprising the steps of holding austenitic stainless steel in a fluorine- or fluoride-containing gas atmosphere with heating prior to carburizing and carburizing the austenitic stainless steel at a temperature not more than 680°C wherein said austenitic stainless steel is stable austenitic stainless steel having 1 to 6 weight % molybdenum or 13 to 25 weight % chromium, wherein a carburized hard layer having corrosion resistance superior to base material forms and austenitic stainless steel products obtained thereby.

## Description

### FIELD OF THE INVENTION

This invention relates to a method of carburizing austenitic stainless steel for hardening its surface and improving corrosion resistance, and austenitic stainless steel products obtained thereby.

### BACKGROUND OF THE INVENTION

Austenitic stainless steel has been widely employed for its superior corrosion resistance property and its capability of decorativeness. Particularly, fasteners such as a bolt, a nut, a screw, a washer and a pin are made of austenitic stainless steel material in view of these properties. Besides, austenitic stainless steel products have been adopted for a variety of machine parts such as various shafts, an impeller, a mold, a spring, a chain and a valve of machinery or equipment in fields of food machinery, chemical plant, nuclear power and the like where high corrosion resistance is required. However, strength itself for most of the above austenitic stainless steel products is improved in an intermediate processing step before a final step to make each figure thereof, which differs from general carbon steel material. For example, crystal structure of the austenitic stainless steel is tightened into closely by cold working or warm working represented by press working, extrusion molding, panting and the like, so-called work hardening, so as to strengthen the material itself. Such improvement of the strength in the intermediate processing step is necessarily limited because there are restrictions to shape the material into a specific figure by the figure such as a bolt or a nut and also to lower cost of a mold in the extrusion molding and the like. Therefore, when surface rigidity or anti seizure is especially demanded on austenitic stainless steel products of fasteners such as a bolt, a nut and a screw, a pump shaft, a bearing and a spring, the following methods are available. ① Hard chromium plating or wet type metal plating such as Ni-P, ② coating such as physical vapor deposition, abbreviated to PVD hereinafter, or ③ hardening treatment by penetration such as nitriding or carburizing.

However, the above methods such as the wet type metal plating or the coating like PVD have drawbacks of shortening product lifetime due to peeling of a coat formed on the surface of the products. Thus, application of hardening treatment by penetration such as carburizing is examined.

Further, nitriding, among the above hardening treatment by penetration, comprises penetrating nitrogen atoms from the surface of austenitic stainless steel material inside thereof so as to form a hard nitrided layer on the surface. However, in this method, the surface hardness of the products is improved, while a vital problem of deteriorating an essential property of anti-corrosion is caused on the other hand. Namely, it is thought that anti-corrosion property deteriorates because chromium atoms (which improve anti-corrosion property) contained in the austenitic stainless steel material itself are consumed as chromium nitrides such as CrN and Cr₂N in the hard nitrided layer and their content therein lowers. Still further, there are problems that the surface blisters, the surface roughness deteriorates, the products are magnetized, or the like.

As the other methods for the above hardening treatment by penetration, there is carburizing. A conventional carburizing method comprises contacting the surface of products with a gas containing carbon so as to invade the carbon atoms into the surface layer and form a hard carburized layer. In this method, carburizing is generally conducted at a temperature not less than 700 °C of an A₁ transformation temperature of iron by considering the permeation speed of carbon atoms and a limit of solid solution. This means, however, that the austenitic stainless steel products have been maintained at a temperature far beyond the recrystallization of iron (N.B. a temperature of recrystallization of iron is about 450°C ) for a long time. As a result, the base material of the hardened austenitic stainless steel by work hardening softens by recrystallization and the like, resulting in remarkable deterioration of the strength of the products, which a great drawback. Moreover, there is another problem that corrosion resistance drastically deteriorates. This is because chromium carbide precipitates in the carburized layer of austentitic stainless steel when the austenitic stainless steel being carburized at such a high temperature, and chromium as solid solution of the austenitic stainless steel is consumed for forming the carbide and their content therein lowers. It is a current situation that carburizing has never been conducted on austenitic stainless steel up to the present accordingly.

The invention can provide a method of carburizing austenitic stainless steel to improve the surface hardness drastically without deteriorating the strength originated from the base material, moreover to form a hard surface layer having corrosion resistance superior to the base material, too, an to provide austenitic stainless steel products obtained thereby.

The invention provides a method of carburizing austenitic stainless steel, with reference to claim 1, comprising maintaining the austenitic stainless steel under a fluorine- or fluoride-containing gas atmosphere with heating prior to carburizing and then carburizing the austenitic stainless steel by setting up a temperature of the carburizing at not more than 680°C wherein said austenitic stainless steel is stable austenitic stainless steel having 1 to 6 weight % molybdenum or 13 to 25 weight % chromium, wherein a carburized hard layer having corrosion resistance superior to bass material forms.

Secondly, the invention provides, with reference to claim 2, a method of carburizing austenitic stainless steel according to claim 1, wherein the carburizing temperature is set within a range of 400 ° to 500°C.

Thirdly, the invention provides, with reference to claim 3, a method of carburizing austenitic stainless steel according to claim 1 or 2, wherein the temperature in a fluorine- or fluoride-containing gas atmosphere in the heating step is set within a range of 250° to 450°C.

Finally, the invention provides, with reference to claim 4, austenitic stainless steel products wherein base material is stable austenitic stainless steel including 1 to 6 weight % molybdenum or 13 to 25 weight % chromium, a surface layer in depth of 5 to 70 µm from the surface is hardened by invasion of carbon atoms so as to be formed into a carburized hard layer whose hardness is 500 to 1050Hv of Micro Vickers hardness, wherein the carburized hard layer is formed by an austenitic phase in which chromium carbide particles do not exist and whose corrosion resistance is superior to the base material.

During a series of studies to improve a technology for better surface hardness of austenitic stainless steel, we came up with an idea that carburizing austenitic stainless steel becomes possible at a temperature not more than an A₁ transformation temperature or steel if pre-treatment with a fluorine- or fluoride-containing gas is conducted before carburizing. During a process based upon this idea, we found out that carburizing becomes possible, which has been regarded as impossible heretofore, if the austenitic stainless steel is treated with a fluorine- or fluoride-containing gas prior to carburizing or at the same time as carburizing. Especially, we also found out that more effective carburizing can be realized at not more than 680°C , preferably not more than 500°C, instead of not less than 700°C employed heretofore. As a result of further studies, we found out that adoption of stable stainless steel as the austenitic stainless steel makes it possible to maintain an austenitic single phase without precipitation of ferrite by the intermediate processing prior to carburizing, which realizes evenly high hardness in the carburized layer with no magnetism. Moreover, we reached the present invention by finding that the resultant carburized layer comes to have corrosion resistance superior to the base material by employing stable stainless steel containing 1 to 6 weight % molybdenum or that containing 13 to 25 weight % Cr, especially among the above stable stainless steel. Stable stainless steel means here stainless steel which completely shows an austenitic phase without ferrite in a view of metallic organization even after being processed into a specific figure at a normal temperature.

At present, the reason why the carburized layer having corrosion resistance superior to the base material is not clear. As a reason, it is thought that a barrier band originated from a C-rich layer formed on the surface layer forms so as to prevent metal ions from dispersing. In this way, a surface layer is formed in 5 to 70 µm depth of the carburized layer, wherein the hardness of the carburized layer is in 500 to 1,050 Hv of Micro Vickers Hardness. Moreover, the carburized layer comprising an austenite phase, which does not precipitate chromium carbide shows corrosion resistance superior to the base material. In addition, there is no problem caused such as surface blisters, deterioration of surface roughness and the like, which have been the conventional problems in nitriding.

It is well known that the above molybdenum is an element for stabilizing ferrite. For this reason, the molybdenum is an obstruction factor against stabilization of an austenite phase of austenitic stainless steel. If a great amount of molybdenum is added, the amount of stabilizing elements for austenite, such as Ni, N, or the like should be increased, resulting in cost increase in raw materials or manufacturing.

The less amount is better. Therefore, it is desirable that 1.0 to 2.5 weight % molybdenum is added to stable stainless steel as a standardized material as SUS316.

In the meantime, the austenite phase where chromium carbide grains do not exist means the austenite phase where crystalline carbides such as Cr₂₃ C₆ , Cr₇C₃ , Cr₃C₂ , or the like cannot be identified by an x-ray diffraction meter commonly used for analyzing crystal structure of metallic material. That is, the austenite phase (τ -phase), a base phase for austenitic stainless steel, has face centered cubic lattice as its crystal structure wherein lattice constant a = 3.59Å , resulting in a specific diffraction peak obtained by the x-ray diffraction. On the other hand, Cr₂₃C₆ is the same centered cubic lattice, however, with lattice constant a = 10.6Å , Cr₇C₃ is trigonal system with lattice constant a = 14.0 Å and c = 4.53 Å , and Cr₃C₂ is prismatic system with lattice constant a = 5.53Å , b = 2.821 Å and c = 11.49Å. Therefore, these chromium carbides differ from the above austenite phase in crystal structure and lattice constant and cause different diffraction peaks from that of the austenite phase. If chromium carbide exists in a carburized hard layer, such peaks that cannot be seen in case of the austenite single phase may emerge. On the other hand, in the carburized hard layer of the present invention, chromium carbide does not exist and carbon atoms invade therein as solid solution so that the lattice of the base austenite phase distorts to form an isotropic austenitic phase, resulting in no emergence of peaks for chromium carbides by x-ray diffraction.

Besides, the stable stainless steel of the present invention means, as mentioned above, such stainless steel that does not produce ferrite metallographically at a normal temperature even after processing into a specific product figure and provides an austenite phase completely. In the figure 4 which shows relationship between Cr equivalent and Ni equivalent (Schaeffler status), Cr equivalent and Ni equivalent of such stainless steel fall within a range (A). In addition, Cr equivalent and Ni equivalent mean values represented by the following formulae (1) and (2) respectively.$\begin{matrix}\begin{matrix}\begin{matrix}\text{Cr equivalent = Cr weight % + Mo weight % + 1.5 x Si weight % + 0.5 x Nb weight %}\end{matrix} \\ \begin{matrix}\text{Ni equivalent = Ni weight % + 30 x C weight % + 0.5 x Mn weight %}\end{matrix}\end{matrix}\end{matrix}$

In addition, in the present invention, evaluation of corrosion resistance is conducted by maintaining samples of carburized materials and untreated materials under the same accelerated corrosive environment and the same conditions and comparing the resultant significant difference indicating corrosion rate. Here, the accelerated corrosion environment means, for example, salt spray, immersion into physiological salt solution, immersion into acid solution such as HCl solution, however, these are not critical, either.

The present invention is now described in further detail.

In the present invention, carburizing after or at the same time as pretreatment by employing fluorine gas is conducted on stable austenitic stainless steel containing 1 to 6 weight % molybdenum or 13 to 25 weight % chromium.

As the stable austenitic stainless steel, there are SUS316, SUS316L and SUS317 which contain 1 to 3 weight % molybdenum, such stainless steel as contains 5 to 6 weight % molybdenum as well as 0.1 to 0.4 weight % N and 22 to 25 weight % Ni as austenite stabilizing elements, austenitic stainless steel material such as SUS304 and SUS310 which contain no molybdenum, 13 to 25 weight % Cr and 8 to 22 weight % Ni, and the like. In the present invention, these are mentioned as base materials.

The amount of the molybdenum to be added into the stable austenitic stainless steel is preferably 1 to 6 weight %, as mentioned above, more preferably 1 to 3 weight % as a viewpoint of cost.

Such stable austenitic stainless steel is employed often for fasteners such as a bolt, a nut, a screw, a washer and a pin. In the invention, austenitic stainless steel products contain chains, a case for a watch, an edge of a spinning shuttle, a minute gear, a knife and machine parts for a wide variety of industries in addition to the above fasteners.

Prior to or at the same time as carburizing, fluorinating treatment is conducted on the above austenitic stainless steel under a fluorine- or fluoride-containing gas atmosphere.

A fluorine- or fluoride-containing gas is employed for this fluorinating treatment. As the above fluorine- or fluoride-containing gas, there are fluorine compound comprising NF₃ , BF₃ , CF₄ , HF, SF₆ , C₂F₆ , WF₆ , CHF₃ , SiF₄ , ClF₃ and the like. These are employed solely or in combination. Besides, a fluorine- or fluoride-containing gas with F in its molecule can be used as the above-mentioned fluorine- or fluoride-containing gas. Also F₂ gas formed by cracking such fluorine compound gas in the heat decomposition device and preliminarily formed F₂ gas are employed as the above-mentioned fluorine- or fluoride-containing gas. According to the case, such fluorine compound gas and F₂ gas are mixed for the use. The above-mentioned fluorine- or fluoride-containing gas such as the fluorine compound gas and F₂ gas can be used independently, but generally are diluted by inert gas such as N₂ gas for the treatment. The concentration of fluorine-fluoride-containing gas itself in such diluted gas should amount to, for example, 10,000 to 100,000ppm, preferably 20,000 to 70,000ppm, more preferably 30,000 to 50,000ppm by capacity. In the light of practicability, NF₃ is the best among the above compound gases. This is because NF₃ has chemical stability and is easy to treat since it is in a state of gas at an ordinary temperature. Such NF₃ gas is usually employed in combination with the above N₂ gas within the above concentration range.

In the invention, first of all, the above-mentioned non-nitrided austenitic stainless steel is held in a furnace under a heated condition in the fluorine- or fluoride-containing gas atmosphere within the above concentration range, and then fluorinated. In this case, the austenitic stainless steel is held with heating at the temperature of, for example, 250° to 600 °C, preferably 280° to 450°C . The holding time of the above-mentioned austenitic stainless steel may be generally within the range of ten or so minutes or dozens of minutes. The passive coat layer, which contains Cr₂O₃ , formed on the surface of the austenitic stainless steel, is converted to a fluorinated layer. Compared with the passive coat layer, this fluorinated layer is thought to be readily penetrated with carbon atoms employed for carburizing. That is, the austenitic stainless steel surface is formed to the suitable condition for penetration of carbon atoms by the above-mentioned fluorination.

Then, carburizing is conducted after the fluorination treatment like the above. In the carburizing, the above austenitic stainless steel itself is heated at not more than 680°C, preferably not more than 600°C, more preferably between 400 ° and 500 °C under a carburizing gas atmosphere, comprising CO and H₂ , or comprising RX [RX components: 23% by volume CO (as abbreviated to vol% hereinafter), 1 vol% CO₂ , 31 vol% H₂ , 1 vol% H₂O, the remainder N₂ ] in a furnace.

Thus, the greatest characteristic in this invention is a low carburizing temperature in which the core part of the austenitic stainless steel may not be softened or solubilized.

In this case, the ratio of CO and H₂ is preferably 2 to 10 vol% for CO and 30 to 40 vol% for H₂ .

The above-mentioned fluorinating and carburizing steps are, for example, taken in a metallic muffle furnace as shown in Fig. 1, that is, the fluorinating treatment is carried out first at the inside of the muffle furnace, and then carburizing treatment is put in practice. In Fig. 1, the reference numeral 1 is a muffle furnace, 2 an outer shell of the muffle furnace, 3 a heater, 4 an inner vessel, 5 a gas inlet pipe, 6 an exhaust pipe, 7 a motor, 8 a fan, 11 a metallic container, 13 a vacuum pump, 14 a noxious substance eliminator, 15 and 16 cylinders, 17 flow meters, and 18 a valve. An austenitic stainless steel product 10 is put in the muffle furnace 1 and fluorinated with heating by introducing the fluorine- or fluoride-containing gas such as NF₃ from the cylinder 16, connected with a duct. The gas is led into the exhaust pipe 6 by the action of the vacuum pump 13 and detoxicated in the noxious substance eliminator 14 before being spouted out. And then, the cylinder 15 is connected with the duct to carry out carburizing by introducing the carburizing gas into the muffle furnace 1. Finally, the gas is spouted out via the exhaust pipe 6 and the noxious substance eliminator 14. Through the series of these operations, fluorinating and carburizing treatments are put in practice.

By this treatment, "carbon" diffuses and penetrates on the surface of austenitic stainless steel so as to form a deep uniform layer. Such a layer realizes drastic improvement in hardness compared with the base material and also retains anti-corrosion property superior to that of the base material, because the layer is in a form wherein a base phase is greatly distorted due to solution of a great amount of carbon atoms.

For example, an SUS316 plate, a typical austenitic stainless steel, is carburized as follows. First the SUS316 plate was introduced into a muffle furnace 1 and was fluorinated at 350°C for 20 minutes under a fluorine- or fluoride-containing gas atmosphere of NF₃ and N₂ (NF₃ : 10 vol%, N₂ : 90 vol%). After exhausting the above a fluorine-or fluoride-containing gas, a carburizing gas of CO, CO₂ and H₂ (38 vol% CO, 2 vol% CO₂ and 60 vol% H₂ ) was introduced into the furnace so that the SUS316 plate was kept at 450 °C in the furnace for 18 hours. As a result, a hard layer having a surface hardness of Hv or 850 (N.B. the core part is Hv of 220 to 230) and a thickness of 20 µm was formed. When this sample was put to the salt spray test (abbreviated to SST hereinafter) according to JIS2371, it did not rust at all over 480 hours. Further, the hard layer was not etched by Billrer reagent (acidic picric acid alcohol solution), which is employed for an anti-corrosion test of a stainless steel organization and was barely etched by aqua regia.
Furthermore, the surface roughness hardly deteriorated, and dimension change by blister and magnetism did not occur in the above sample.

As a result of further studies by varying the combination of various kinds of austenitic stainless steel plates, carburizing temperatures and the like, it was found out that the core of austenitic stainless steel easily softens and also anti-corrosion property of the hard layer drastically deteriorates when a carburizing temperature is over 600 °C . Namely, it was found out that from a viewpoint of anti-corrosion property, a carburizing temperature is preferably not more than 600°C, more preferably not more than 500°, which brings about a better result. As mentioned above, a more preferable carburizing temperature is 400 ° to 500°C .

In the present invention, when a carburizing temperature increases, especially surpasses 450 °C, a phenomenon that carbide such as Cr₂₃C₆ precipitates on the surface of the hard layer although it is a very small amount. However, even in this case, if a carburized article is soaked into strong acid such as HF-HNO₃ solution, HCl-HNO₃ solution or the like to remove the above precipitation, anti-corrosion property higher than the base material and usually excellent surface hardness not less than Hv of 850 in Vickers hardness can be retained.

Namely, in thus carburized austenitic stainless steel products, the carburized hard layer formed on the surface becomes black due to carburizing and the outermost layer may form into an iron inner oxide layer due to the presence of a small amount of oxygen atoms in the carburizing atmosphere, according to a case. However, the removal of the inner oxide layer, as mentioned before, can be conducted by soaking into strong acid such as HF-HNO₃ solution and HCl-HNO₃ solution so as to remove the above deposit. Thereby, corrosion resistance superior to that of the base material and high surface hardness not less than 850Hv of Vickers hardness can be maintained. Austenitic stainless steel products wherein the inner oxide layer is removed by the above treatment turn to show glossiness as the same as that before being carburized.

A chart C of Fig. 2 shows an x-ray diffraction chart of an SUS316 article which is carburized at 480 °C and then soaked into strong acid of 5 vol% HF and 15 vol% HNO₃ concentration for 20 minutes, wherein no carbide was observed.

This is further described in detail. As a result of visual observation on the surface of products after being carburized, it was found out that a dark color layer exists in depth of 2 to 3 µm in the outermost layer. This layer was identified as an iron inner oxide layer by an x-ray diffraction method. This means that carburizing ${\text{(2CO → CO}}_{\text{2}} \text{+C)}$and oxidation of ${\text{Fe (4CO}}_{\text{2}} {\text{+3Fe → 4CO+Fe}}_{\text{3}} {\text{O}}_{\text{4}} \text{)}$may coexist at the same time under the atmosphere containing CO at a temperature between 400 ° and 500°C so that the above inner oxide layer was formed. Such an iron inner oxide layer cannot be seen in conventional carburizing methods at not less than 700°C .

Further, in detail, when a socket bolt and a washer of SUS316L (C=0.02wt%, Cr=17.5wt%, Ni=12.0wt% and Mo=2.0wt%) were carburized at 480°C for 12 hours, the hard layer depth was 30 µm and the surface hardness showed 910Hv of Micro Vickers Hardness, however, the surface color was black. Consecutively, these black colored carburized articles were soaked into solution of 5 vol% HF - 25 vol% HNO₃ heated to 50 °C for 20 minutes and then conducted with soft blast so that a socket bolt and a washer, which showed glossy appearance as the same as those before being carburized, could be obtained.

These were subjected to JIS 2371 Salt Spray Test so that no rusts were caused in 2,000 hours. Further, corrosion resistance superior to the base material was confirmed in organic and inorganic acid resistance tests and an elusion test for physiological salt solution.

Thus, according to the carburizing of this invention, the articles with such a treatment retain excellent anti-corrosion property, which is thought to be due to the following two reasons. Since fluorinating treatment is conducted prior to carburizing, a low carburizing temperature not more than 680 °C can be realized. By this carburizing at a low temperature, chromium element, which is thought to work for improving anti-corrosion property, in austenitic stainless steel is difficult to precipitate and fix as carbide such as Cr₇C₂ , Cr₂₃C₆ or the like and then the volume of fixed precipitation lowers, whereby much chromium element remains in the austenitic stainless steel. In this way, deterioration in corrosion resistance of the base material can be prevented. This is clear by comparing an x-ray diffraction results for an SUS316 article (an x-ray diffraction chart shown in Fig. 3), which was fluorinated under a fluorine- or fluoride-containing gas of 10 vol% NF₃ and 90 vol% N₂ at 300 °C for 40 minutes and then carburized under a carburizing gas of 32 vol% CO, 3 vol% CO₂ and 65 vol% H₂ at 600 °C for 4 hours, and for an SUS316 article (an x-ray diffraction chart B shown in Fig. 2), which was fluorinated in the same way and carburised at 450 °C for 16 hours, with an x-ray diffraction result for an SUS316 article (an x-ray diffraction chart A shown in Fig. 2), which was untreated. That is, a peak of Cr₂₃C₆ is sharp and high in articles carburized at 600 °C in Fig. 3. This means that the above chromium carbide precipitates relatively much while less chromium element remains in austenitic stainless steel. On the other hand, a peak of Cr₂₃C₆ can be hardly identified in carburizing at 450 °C in Fig. 2 (B). This means that the precipitation of the above chromium carbide is extremely low while more chromium element remains in austenitic stainless steel, resulting in high anti-corrosion property. Secondly, by employing stable stainless steel containing 1 to 6 weight % molybdenum or 13 to 25 weight % chromium, a barrier band originated from a C-rich layer formed on the surface layer forms so as to prevent metallic ions from dispersing and also molybdenum may contribute to improvement in acid resistance of austenitic stainless steel, resulting in corrosion resistance of the carburized layer superior to the base material.

Furthermore, an improvement in hardness of carburized articles is thought to be attributed to occurrence of austenite lattice distortion by penetration of carbon atoms. It is clear that austenite lattice distortion is caused in a carburized article in Fig. 2 (B) and (C), because austenite phase peak position (B shown in Fig. 2) of a carburized article at 450°C and that (C shown in Fig. 2) of a carburized and acid-treated article at 480 °C according to an x-ray diffraction shift to low angle side (left side) from that (A shown in Fig. 2) of untreated SUS316 article. In addition, the above x-ray diffraction was conducted by RINT1500 device at 50KV, 200mA and Cu target.

In addition, since the diffusion speed of C in austenitic organization is relatively slow in case of a low temperature region not more than 500°C , it takes a considerable time to obtain a thick layer. For example, the above carburized hard layer on SUS316L series, in which a hard layer becomes the thickest, becomes 37 µm with treatment at 490 °C for 12 hours and becomes only 49 µm with additional treatment for another 12 hours. To obtain a hard layer in 70 µm depth, it takes not less than 70 hours. Such long-time treatment is not economical. Even in drill tapping, which requires a hard layer as thick as possible, it is possible to drill SPCC (Steel Plate, Cold Coiled) of 2.3t with a hard layer in 40 µm depth, whereby a useful hard layer can be obtained in suitable time with economical efficiency. In addition, when carbon concentration in the above carburized layer is set at or around 2.0 weight % as an upper limit, the effect of improving surface hardness can be increased.

### EFFECT OF THE INVENTION

As mentioned hereinbefore, carburizing austenitic stainless steel according to the invention realizes a low carburizing temperature not more than 680°C because the austenitic stainless steel is kept being heated under the fluorine- or fluoride-containing gas atmosphere prior to or at the same time as carburizing. Therefore, high surface hardness as well as anti-corrosion property superior to the base material can be realized without deteriorating high processability inherent in austenitic stainless steel itself. In addition, since the surface hardness is improved thanks to the above carburizing, any inconveniences such as surface roughness caused by nitriding, dimension inaccuracy by blister and magnetization in austenitic stainless steel itself are not occurred at all.

Thus obtained austenitic stainless steel products have a hard layer in depth of 5 to 70 µm which is formed into a carburized layer by invasion of carbon atoms of 500 to 1,180Hv Micro Vickers Hardness, preferably 500 to 1,050Hv. Further, since chromium carbide are not deposited in the carburized hard layer and formed by an austenitic phase, the obtained products show corrosion resistance superior to the base material due to formation of C-rich band of the outermost layer. Therefore, thus obtained products are useful for fasteners such as a bolt, a nut and a screw as well as a variety of machine parts for general industrial fields such as various shafts, an impeller, a bearing, springs, and valve parts. In addition, especially, these are promising as materials for machine parts employed in fields of food machinery, chemical plant and semiconductor industry.

### BRIEF DESCRIPTION OF THE DRAWINGS

Fig. 1 schematically shows a construction of a furnace for carrying out carburizing according to the invention,
Fig. 2 shows curves of each x-ray diffraction on an untreated SUS316 article, a carburized SUS316 plate at 450 °C and an SUS316 plate, which was carburized at 480 °C and treated with strong acid,
Fig. 3 shows a curve of x-ray diffraction on an SUS316 plate which was carburized at 600 °C ; and
Fig. 4 shows the relationship between Cr equivalent and Ni equivalent.

The following example is further illustrative of the invention.

### EXAMPLE 1

Plural rolled plates (2.5t x 15 x 15) of SUS316 (Cr content: 17 weight %, Ni content: 13.5 weight %, Mo content: 2.5 weight %, C content: 0.07 weight % and Fe content: the remainder) and plural rolled plates (2.5t x 15 x 15) of SUS304 (Cr content: 18.5 weigh %, Ni content: 8.5 weight %, C content: 0.08 weight % and Fe content: the remainder) were prepared as examples. The core hardness of these materials were Hv=220 to 230 for SUS316 materials and Hv=170 to 180 for SUS304 materials. These materials were fluorinated by blowing a gas mixture of 20 vol% NF₃ and N₂ for the remainder into a furnace shown in Fig. 1 for 15 minutes when being heated to 320°C therein, purged with N₂ gas and heated to 480°C . Subsequently, a carburizing gas of 31 vol% H₂ , 21 vol% CO, 1 vol% CO₂ and the remainder of N₂ was charged therein. The materials were maintained therein for 15 hours so as to be carburized. Consecutively, such treated materials were dipped into solution of 3 vol% HF and 15 vol% HNO₃ , heated to 55°C, for 30 minutes to be cleansed.

As a result of measuring depth and hardness of these hard layers, the depth and hardness for SUS316 were 32 µm and Hv=980, while those for 304 were 28 µm and Hv=1,080 respectively.

As samples, plates of the above carburized SUS316 materials, SUS304 materials and also both untreated materials were dipped into solution of 5 vol% HCl, heated to 50°C and maintained for 3 hours. Subsequently, each elusion concentration of metallic ions was determined by atomic absorption analysis for evaluation of corrosion resistance. The results are shown in the following table 1.

**TABLE 1**

| | TIME (H) | TEMPERATURE (°C) | ELUSION CONCENTRATION OF METALLIC IONS (ppm) | | |
|---|---|---|---|---|---|
| | | | Fe | Ni | Cr |
| SUS316 | | | | | |
| Untreated | 3 | 50 | 198 | 30 | 40 |
| Carburized | 3 | 50 | 3.6 | 0.6 | 0.4 |

| SUS304 | | | | | |
|---|---|---|---|---|---|
| Untreated | 3 | 50 | 720 | 150 | 180 |
| Carburized | 3 | 50 | 150 | 33 | 28 |

As clear from the above results, the carburized SUS316 sample showed corrosion resistance drastically superior to the untreated sample (i.e., the base material). Besides, the carburized 304 sample showed corrosion resistance superior to the untreated sample.

## Claims

1. A method of carburizing austenitic stainless steel comprising the steps of holding austenitic stainless steel in a fluorine- or fluoride-containing gas atmosphere with heating prior to carburizing and carburizing the austenitic stainless steel at a temperature not more than 680 °C wherein said austenitic stainless steel is stable austenitic skinless steel having 1 to 6 weight % molybdenum or 13 to 25 weight % chromium, wherein a carburized hard layer having corrosion resistance superior to base material forms.

2. A method of carburizing austenitic stainless steel according to claim 1, wherein the carburizing temperature is set within a range of 400° to 500°C .

3. A method of carburizing austenitic stainless steel according to claim 1 or 2, wherein the temperature in fluorine- or fluoride-containing gas atmosphere in the heating step is set within a range of 250° to 450°C .

4. Austenitic stainless steel products wherein base material is stable austenitic stainless steel including 1 to 6 weight % molybdenum or 13 to 25 weight % chromium, a surface layer in depth of 5 to 70 µm from the surface is hardened by invasion of carbon atoms so as to be formed into a carburized hard layer whose hardness is 500 to 1050Hv of Micro Vickers hardness, wherein the carburized hard layer is formed by an austenitic phase in which chromium carbide particles do not exist and whose corrosion resistance is superior to the base material.
